# EUROPEAN PATENT SPECIFICATION

(11) **EP 0 788 535 B1**
(45) Date of publication and mention of the grant of the patent: **03.05.2000**
(21) Application number: 95938911.5
(22) Date of filing: 25.10.1995
(51) Int. Cl.: C10M 129/00, C10M 129/40, C10M 129/58, C10M 129/93

(54) **NOVEL COBALT CONTAINING DEPOSIT CONTROL ADDITIVES**
KOBALT ENTHALTENDE ADDITIVE ZUR KONTROLLE VON ABLAGERUNGEN
NOUVEAUX ADDITIFS A BASE DE COBALT REGULANT LES DEPOTS

(30) Priority: 25.10.1994 US 328209
(43) Date of publication of application: 13.08.1997
(73) Proprietor: EXXON RESEARCH AND ENGINEERING COMPANY, Florham Park, New Jersey 07932-0390 (US)
(72) Inventor: HOLT, David, G., L., Brights Grove, Ontario N0N 1C0 (CA); FRANCISCO, Manuel, A., Washington, NJ 07882 (US)
(74) Representative: Fletcher Watts, Susan J.
(86) International application number: US9513840
(87) International publication number: WO9612779

(56) References cited:
- EP-A- 0 444 830
- FR-A- 2 372 222
- GB-A- 772 029
- US-A- 3 360 467
- US-A- 3 412 028

## Description

### Field of the Invention

The present invention relates to novel lube oil base stock compositions containing deposit control additives.

### Background of the Invention

Copper is a common lube oil antioxidant additive. However, it forms deposits at higher temperatures. As a result additives and methods for increasing the lifetime of copper antioxidants and for retarding their degradation and resulting deposit formation would be desirable. The present invention addresses these needs. FR-A-2 372 222 and GB-A-772 029 disclose the use of copper and cobalt as lubricating oil additives.

### Summary of the Invention

The present invention provides for formulated lubricating oil compositions, comprising a base stock of lubricating viscosity, a copper containing antioxidant and a deposit control enhancing amount of an oil soluble or oil dispersible cobalt containing compound.

The present invention also provides for a method of controlling deposit formation in an engine lubricating system, comprising adding a deposit control enhancing amount of an oil soluble or oil dispersible cobalt containing compound to a base oil of lubricating viscosity formulated with a copper containing antioxidant.

The present invention may suitably comprise, consist or consist essentially of the elements disclosed herein and may be practiced in the absence of any element not disclosed herein as required.

### Detailed Description of the Invention

The present invention provides for a method of controlling deposits, i.e. retarding deposit formation and buildup, in internal combustion engines by enhancing the performance of a certain base stocks containing copper containing antioxidants, with the addition of cobalt containing compounds as disclosed in claim 1. The invention also provides for novel formulated oil and additive compositions related thereto. As a benefit the life of the copper containing antioxidant and the formulated oil can be extended, as disclosed in claim 7 and the use of cobalt and copper soluble compound to enhance the control of deposit formation disclosed in claim 8.

The starting materials disclosed herein may be made by methods known in the art or obtained from commercial sources.

Generally copper containing compounds and the cobalt containing compounds are individually present in a minor amount by weight percent of the compound to a major amount of the oil. The term "minor amount" as used herein is intended to mean that amount is less than 50% by weight of the composition. The term "major amount" is intended to mean that amount is more than 50% by weight of the composition.

The copper antioxidant should be present in a hydrocarbon, preferably oil soluble or dispersible form. These antioxidants are of the type and are present in amounts typically used as lube additives for internal combustion engines as these represent an economical and readily available source of the materials. Suitable examples include copper naphthenates, oleates and polyisobutylene succinic anhydride ("PIBSA") compounds. Thus, these amounts may vary with the particular formulation without affecting the present invention.

The cobalt containing compounds that produce the synergistic effect of enhancing deposit control in formulated oils having copper containing antioxidants therein should be present in a hydrocarbon, preferably oil soluble or dispersible form. Thus, any source of cobalt is acceptable provided that it is oil soluble or dispersible. Examples include oil soluble cobalt salts such as cobalt naphthenates, or cobalt stearates and inorganic cobalt salts in combination with suitable dispersants or surfactants, for example cobalt PIBSA or cobalt acetylacetonate ("acac"). It is desirable that the cobalt containing compound be compatible with the copper containing compound as well as the base stock or formulated oil to which it is added in order to achieve the synergistic effect of retarding deposit formation and extending the life of the copper antioxidant and formulated oil. The cobalt is present in an amount sufficient to enhance deposit control performance, i.e., to retard deposit formation and, thus, extend the life of the lube oil containing the copper antioxidant. This amount, for lube applications, typically is a minor amount of cobalt metal, from about 10-1000 ppm, preferably about 50-500 ppm, more preferably about 75-200 ppm, as determined on the basis of the amount of the metal present in the formulated compositions.

The foregoing may be added to the base and formulated oils by means well known in the art.

As used herein the term hydrocarbon or oil "soluble" and "dispersible" means that the material is soluble or stably dispersible in hydrocarbons, preferably oils of lubricating viscosity, that are liquid at temperatures found in the environments at which the formulated oils are typically used. The term "stably dispersible" means that the material is capable of being dispersed in the hydrocarbon or oil to an extent that allows it to function in its intended manner. Thus, for example in lube oil formulations, a copper antioxidant or the cobalt antioxidant is hydrocarbon or oil soluble or dispersible if it is capable of being dissolved, dispersed or otherwise suspended in the oil in a manner sufficient to allow the oil to function as a lubricant. Detergents such as neutral and/or overbased blends of calcium sulfonated detergents and dispersants such as borated PIBSA-PAM may be used to achieve oil solubility or dispersibility.

The base oils employed in the lubricant compositions according to the invention may be any base oil suitable for the intended use of the lubricant. Thus, the base oil may be, for example, a conventionally refined mineral oil, an oil derived from coal tar or shale, a vegetable oil, an animal oil, a hydrocracked oil, or a synthetic oil, or a mixture of two or more of these types of oils. Examples of synthetic oils include hydroisomerised paraffins, polyalpha-olefins, polybutenes, alkylbenzenes, polyglycols, esters such as polyol esters or dibasic carboxylic acid esters, alkylene oxide polymers, and silicone oils. The viscosity of the base oil depends upon the intended use, but generally is in the range of from 3 to 20cSt at 100°C.

The present invention also permits the use of other additives in the oil compositions. These other additives include such conventional additive types as viscosity modifiers, extreme pressure agents, corrosion-inhibiting agents, pour point depressants, color stabilizing agents, anti-foam agents, and other such additive materials known generally to those skilled in the art of formulating lubricants.

It is expected that the benefits described herein can be achieved over the range of amounts and types of copper containing antioxidants generally used as lube oil additives.

It is expected that similar benefits could be obtained in fuels.

The present invention may be exemplified by reference to the following examples:

### Example 1 -- Inclined Panel Deposit Test

The effect of the presence of cobalt containing compounds in a lube oil formulated with a copper containing antioxidant was evaluated using the Inclined Panel Deposit Test (IPDT). The beneficial and synergestic effect on engine deposit formation of adding cobalt containing compounds to base oils formulated with copper containing antioxidants can be determined by measuring the buildup of deposits during the course of the test. The beneficial effect of cobalt addition is evidenced by smaller amounts of deposit formation.

The IPDT is a bench test that simulates piston deposit formation during engine operation. 35 ml of oil was heated to 150°C and run down a metal panel heated to 308°C at a 2 degree angle. The oil was then pumped through a sump back onto the panel. The oil was exposed to a synthetic blow-by gas throughout the 2 hour duration of the test. The panel was cooled and washed with heptane. The rating figure (demerit) value indicates the amount of deposition on the plate. A higher number (greater demerit) indicates greater deposit formation, with 10 being the highest and zero the lowest.

Table 1 shows the results of the IPDT using a commercially available mineral oil base stock formulated with commercially available additive package containing copper PIBSA and a monofunctional olefin copolymer VI improver, borated PIBSA pour point depressant, calcium sulfonate overbased detergent, neutral calcium sulfonate detergent, nonyl phenyl sulfide antioxidant, ZDDP antiwear, molybdenum dithiocarbonate antiwear additive alone (Run 1) and in the presence of cobalt additive (Run 2) demonstrating the synergistic effect of adding cobalt in copper antioxidant systems. A comparative example demonstrating the deterioration of results upon addition of cobalt to a commercially available diphenyl amine and hindered phenolic antioxidant additive package is shown in Table 2.

**TABLE 1**

| INCLINED PANEL DEPOSIT TEST | | |
|---|---|---|
| | FORMULATED OIL | RESULT (DEMERITS) |
| (1) | Lube base stock formulated with copper antioxidant* | 6.4 |
| | | |
| (2) | Lube base stock formulated with copper antioxidant* + 100 ppm cobalt antioxidant** | 3.4 |

| | | |
|---|---|---|
| * 0.3 wt% copper PIBSA antioxidant | | |
| ** 0.17 wt% cobalt naphthenate | | |

**TABLE 2**

| INCLINED PANEL DEPOSIT TEST (COMPARATIVE DATA) | | |
|---|---|---|
| FORMULATED OIL | | RESULT (DEMERITS) |
| (1) | Lube base stock formulated with diphenyl amine and hindered phenolic antioxidant | 2.4 |
| | | |
| (2) | Lube base stock formulated with diphenyl amine and hindered phenolic antioxidant + 100 ppm cobalt | 4.0 |

## Claims

1. A formulated internal combustion engine lubricating oil composition, comprising a base engine oil of lubricating viscosity, a copper containing antioxidant, and a deposit control enhancing amount of an oil soluble or oil dispersible cobalt containing compound, which provides from 10 to 1000 ppm by weight of cobalt metal in the formulated lubricant composition.

2. The composition of claim 1 wherein the amount of the cobalt containing compound is from 50 to 500 ppm by weight based on the amount of cobalt metal in the formulated lubricant composition.

3. The composition of claim 1 or 2 wherein the cobalt containing compound is selected from cobalt naphthenates, cobalt stearates, cobalt polyisobutylene succinic anhydrides and cobalt acetylacetonates.

4. The composition of any preceding claim wherein the copper containing antioxidant is selected from copper naphthenates, oleates, stearates and polyisobutylene succinic anhydrides.

5. The composition of any preceding claim further comprising at least one agent selected from a dispersant and a detergent.

6. The composition of any preceding claim further comprising at least one additive selected from antiwear agents, viscosity modifiers, extreme pressure agents, antifoam agents, pour point depressants, and colour stabilizing agents.

7. A method of controlling deposit formation in an internal combustion engine lubricating system, comprising: combining a deposit control enhancing amount of from 10 to 1000 ppm by weight based on the amount of cobalt metal in the formulated lubricant composition of an oil soluble or oil dispersible cobalt containing compound with a base engine oil of lubricating viscosity formulated with a copper containing antioxidant.

8. Use of an oil soluble or oil dispersible cobalt containing compound to enhance the control of deposit formation in an internal combustion engine lubricating system, which lubricating system comprises a base engine oil of lubricating viscosity and a copper containing antioxidant.

## Patentansprüche

1. Formulierte Schmierölzusammensetzung für Verbrennungsmotoren, die Basismotoröl mit Schmierviskosität, kupferhaltiges Antioxidans und eine die Kontrolle von Ablagerungen erhöhende Menge öllösliche oder öldispergierbare kobalthaltige Verbindung umfaßt, die 10 bis 1000 Gew.ppm Kobaltmetall in der formulierten Schmierstoffzusammensetzung liefert.

2. Zusammensetzung nach Anspruch 1, bei der die Menge an kobalthaltiger Verbindung 50 bis 500 Gew.ppm beträgt, bezogen auf die Menge an Kobaltmetall in der formulierten Schmierstoffzusammensetzung.

3. Zusammensetzung nach Anspruch 1 oder 2, bei der die kobalthaltige Verbindung ausgewählt ist aus Kobaltnaphthenaten, Kobaltstearaten, Kobalt-Polyisobutylenbernsteinsäureanhydriden und Kobaltacetylacetonaten.

4. Zusammensetzung nach einem der vorhergehenden Ansprüche, bei der das kupferhaltige Antioxidans ausgewählt ist aus Kupfernaphthenaten, -oleaten, -stearaten und -Polyisobutylenbernsteinsäureanhydriden.

5. Zusammensetzung nach einem der vorhergehenden Ansprüche, die ferner mindestens ein Mittel ausgewählt aus Dispergiermittel und Detergens umfaßt.

6. Zusammensetzung nach einem der vorhergehenden Ansprüche, die ferner mindestens ein Additiv ausgewählt aus Antiverschleißmitteln, Viskositätsmodifizierungsmitteln, Extremdruckmitteln, Antischaummitteln, Stockpunktsenkungsmitteln und Farbstabilisierungsmitteln umfaßt.

7. Verfahren zur Kontrolle der Bildung von Ablagerungen im Schmiersystem eines Verbrennungsmotors, bei dem eine die Kontrolle von Ablagerungen erhöhende Menge von 10 bis 1000 Gew.ppm, bezogen auf die Menge an Kobaltmetall in der formulierten Schmierstoffzusammensetzung, einer öllöslichen oder öldispergierbaren kobalthaltigen Verbindung mit einem Basismotoröl mit Schmierviskosität kombiniert wird, das mit kupferhaltigem Antioxidans formuliert ist.

8. Verwendung von öllöslicher oder öldispergierbarer kobalthaltiger Verbindung zur Erhöhung der Kontrolle der Bildung von Ablagerungen im Schmiersystem eines Verbrennungsmotors, wobei das Schmiersystem Basismotoröl mit Schmierviskosität und kupferhaltiges Antioxidans umfaßt.

## Revendications

1. Composition d'huile lubrifiante formulée de moteur à combustion interne, comprenant une huile de moteur de base de viscosité lubrifiante, un antioxydant contenant du cuivre et une quantité, améliorant le contrôle de formation de dépôts, d'un composé contenant du cobalt, soluble ou dispersable dans les huiles, qui apporte 10 à 1000 ppm en poids de cobalt métallique dans la composition lubrifiante formulée.

2. Composition selon la revendication 1, dans laquelle la quantité de composé contenant du cobalt est de 50 à 500 ppm en poids par rapport à la quantité de cobalt métallique dans la composition lubrifiante formulée.

3. Composition selon la revendication 1 ou 2, dans laquelle le composé contenant du cobalt est choisi parmi les naphténates de cobalt, les stéarates de cobalt, les anhydrides polyisobutylènesucciniques de cobalt et les acétylacétonates de cobalt.

4. Composition selon l'une quelconque des revendications précédentes, dans laquelle l'antioxydant contenant du cuivre est choisi parmi les naphténates, les oléates, les stéarates et les anhydrides polyisobutylènesucciniques de cuivre.

5. Composition selon l'une quelconque des revendications précédentes, comprenant par ailleurs au moins un agent choisi parmi un dispersant et un détergent.

6. Composition selon l'une quelconque des revendications précédentes, comprenant par ailleurs au moins un additif choisi parmi les agents anti-usure, les modificateurs de viscosité, les agents de pression extrême, les agents anti-mousse, les abaisseurs de point d'écoulement et les agents stabilisateurs de couleur.

7. Procédé de contrôle de la formation de dépôts dans un système lubrifiant de moteur à combustion interne, comprenant la combinaison d'une quantité, améliorant le contrôle de la formation de dépôts, de 10 à 1000 ppm en poids, par rapport à la quantité de cobalt métallique dans la composition lubrifiante formulée, d'un composé contenant du cobalt, soluble ou dispersable dans les huiles, avec une huile de moteur de base de viscosité lubrifiante formulée avec un antioxydant contenant du cuivre.

8. Utilisation d'un composé contenant du cobalt, soluble ou dispersable dans les huiles, pour améliorer le contrôle de la formation de dépôts dans un système lubrifiant de moteur à combustion interne, ledit système lubrifiant comprenant une huile de moteur de base de viscosité lubrifiante et un antioxydant contenant du cuivre.
